

April 29, 1969

N. P. DEMAS

3,441,332

METHOD FOR GETTERING COMPLETED GAS FILLED LAMPS  
AND THE PRODUCT RESULTING THEREFROM  
Filed July 15, 1966



INVENTOR  
NICKOLAS P. DEMAS  
BY *Eyre, Mann & Lucas*  
ATTORNEYS

1

3,441,332

## METHOD FOR GETTERING COMPLETED GAS FILLED LAMPS AND THE PRODUCT RESULTING THEREFROM

Nickolas P. Demas, Cranford, N.J., assignor, by mesne assignments, to Wagner Electric Corporation, South Bend, Ind., a corporation of Delaware

Filed July 15, 1966, Ser. No. 565,616

Int. Cl. H01j 9/38

U.S. Cl. 316—26

4 Claims

### ABSTRACT OF THE DISCLOSURE

A gas filled incandescent lamp with a getter spot is formed by heating the sealed glass envelope of the lamp, energizing the filament of the lamp so that it is electron-emissive, contacting the heated portion of the lamp envelope with a disassociated alkali metal compound, and causing the conduction of alkali metal ions through the glass by applying a voltage between the filament and the disassociated alkali metal compound, thereby forming a getter spot corresponding to the area of contact of the alkali metal compound.

The present invention relates to the manufacture of lamps and comprises an improved method for manufacturing incandescent gas filled lamps. By utilizing the method of the invention, it is possible to introduce a getter material into a sealed gas filled lamp after all other steps in the production of the lamp are completed. The resultant lamp product is of an improved quality and increased commercial value. The invention also includes the gettered lamp produced by this new method of manufacture.

One problem which arises during the manufacture of incandescent gas filled lamps is the premature blackening of the lamp envelope due to a chemical attack on the lamp filament by impurities in the gas fill such as oxygen, hydrogen, carbon dioxide and water. These impurities combine with the tungsten in the lamp filament to cause the formation of tungsten deposits on the interior of the lamp envelope.

One known method of preventing the undesirable tungsten deposits and also the resulting blackening of the lamp is to introduce an alkali getter material into an unsealed lamp at a preliminary stage in its manufacture. As described in my Patent No. 3,189,395, "Method of Making Incandescent Lamps," a sodium getter can be introduced into an evacuated unsealed lamp by electrolytic conduction of sodium through the lamp wall. With the application of a small voltage across the incandescent lamp filament and a molten sodium bath which is brought in contact with the heated lamp envelope, sodium ions will pass directly through the lamp bulb. The ions become sodium atoms upon combination with electrons emitted from the lamp filament and the atoms are quickly vaporized due to the high temperature and sub-atmospheric pressure in the envelope. The vaporized sodium solidifies on any cool portion of the envelope to form a getter spot. All impurities are absorbed by the sodium and any desired amount of neon or argon gas can be introduced into the envelope prior to the sealing thereof.

In this regard, it has heretofore been impossible to remove a completed gas filled lamp from an assembly line after the final step in its manufacture and successfully introduce an absorbent alkali getter material directly into the lamp by electrolytic conduction. It is now believed that the electrolytic process breaks down during the gettering of a gas filled lamp and that this breakdown is due to a polarization effect which occurs within the lamp envelope. The polarization effect results from the com-

2

bination of electrons emitted by the lamp filament with ions of insert gas within the envelope. Since the alkali metal ions which have migrated through the glass are thus not neutralized, they maintain their positive charge and prevent further migration of alkali metal ions from the supply. Discovery of this polarization effect has paved the way for the improved method of gettering lamps which is the subject of the present invention.

In accordance with the method of the present invention, the above mentioned polarization effect is overcome and an alkali metal is electrolytically passed into a completed lamp which contains a quantity of inert gas. In practicing the method of the invention, a portion of the gas filled envelope is heated to a temperature which is sufficient to make the glass electrically conductive but which does not soften the glass. In order to provide a supply of an alkali metal from which a getter deposit can be formed, a rod or probe is dipped into a molten compound of the alkali metal. The quantity of alkali metal compound which remains on the probe after it is withdrawn forms the supply of alkali metal. The probe with the alkali metal compound thereon is then brought into contact with the heated portion of the lamp. Electrons are emitted by the lamp filament when a source of potential is connected across the filament or by other means such as cold cathode emission. The electrons are emitted into the interior portion of the envelope which confines an inert gas such as argon or neon. A second source of potential is connected across the lamp filament and the probe carrying the supply of alkali metal compound. The voltage of this source is critical and must be large enough to overcome any polarization which is taking place in the lamp envelope but small enough to permit orderly and controlled electrolytic conduction of the alkali metal through the envelope of the lamp. When a getter deposit of alkali metal has formed on a portion of the interior of the lamp envelope adjacent to the outer envelope surface which is in contact with the probe carrying the supply of alkali metal compound, the second source of potential can be disconnected. The boundaries and location of the getter deposit are determined by the dimensions of the heated area of the lamp, the surface area of the alkali metal supply carried by the probe and the position of the probe as it is held in contact with the lamp envelope during the electrolysis. The gettered lamp which is formed by practicing this novel method is also included in the present invention.

The present improved method of gettering completed gas filled lamps affords several advantages over the prior art due to the fact that a sealed rather than an unsealed evacuated lamp is employed. With the present method, the getter material can be deposited directly on the sealed envelope wall without the vaporization of the getter material which results when unsealed lamps are used. Consequently, pressure control within the lamp envelope during the gettering process is no longer required and that step in the lamp manufacture process can be eliminated. Furthermore, by utilizing a sealed lamp envelope, the problem of loss of getter material by vaporization through the unsealed end of the lamp is avoided. Also, when the lamp is sealed, getter material cannot escape from the confines of the lamp to foul the machinery used in the process. Another advantage of the invention is that the size and location of the getter spot can be closely controlled without subjecting any portion of the lamp envelope to a cooling process.

For a better understanding of the invention, reference may be had to the accompanying drawings in which:

FIG. 1 is a diagram representing a stage in the process wherein a portion of the envelope of a completed gas filled lamp is heated to render it electrically conductive;

FIG. 2 is a diagram representing a succeeding stage in the process wherein alkali metal ions are passed through

the heated portion of the lamp envelope by electrolytic conduction; and

FIG. 3 is a bottom view of a gettered cartridge lamp produced by the method of the present invention.

In FIG. 1 a gas filled cartridge lamp is shown at 2 which comprises an elongated lamp envelope 4, a lamp filament 6 positioned within the envelope and lamp leads 8 which are connected to the lamp filament 6 at connection point 9 and extend partially outside the envelope. The lamp leads 8 are sealed in position by crimping a portion 10 of the lamp envelope 4 during its manufacture, as best seen in FIG. 3. The envelope can be filled with argon gas at a pressure of about 400 mm. Hg at room temperature prior to the sealing thereof.

It should be noted that prior to the commencement of the gettering process, the cartridge lamp 2 is a complete and operative lamp. The primary purpose of introducing a getter into the lamp is to absorb any abnormal impurities which are present within the envelope. In addition however when the getter material has performed its absorbing function, it assumes a chalk-like appearance which provides visual evidence of the purity of the atmosphere within the lamp and thereby guarantees the performance and long life of the lamp.

During the process of the invention, the lamp 2 is mounted by conventional means (not shown) and a portion of the lamp envelope is heated, as by a flame from a burner 14 as shown in FIG. 1. If the lamp envelope is made of lime or soda glass, a heating temperature of 300° C. will cause the envelope to become electrically conductive without softening the glass.

In FIG. 2 a probe 15 is shown as it is held in contact with the heated portion of the lamp envelope. An end portion 16 of the probe 15 having been previously dipped into a source 17 of a molten alkali metal compound provides a supply of alkali metal which is to be passed into the lamp.

To eliminate the step of heating the glass envelope and the use of a probe, a portion of the envelope can be dipped directly into the source 17 of alkali metal compound. In this case, the glass is heated by the molten compound to a temperature which makes the glass electrically conductive, but the area of sodium deposition is less easy to control.

The molten alkali metal compound is preferably a eutectic mixture of sodium nitrate and sodium nitride. For the purpose of explanation, sodium nitrate,  $NaNO_3$ , will be used in describing the operation of the process but it is to be understood that other alkali metal compounds and combinations thereof can be employed if the same alkali metal is also present in the glass walls of the lamp.

The probe 15, or the source 17 when no probe is used, is connected through a switch 18 to the positive terminal of a source of potential 20, the negative terminal of which is connected to the lamp lead 8. A second source of potential 22 is placed across the lamp leads 8 and the filament 6 to thereby heat the filament to incandescence and initiate the emission of electrons. Since molten  $NaNO_3$  dissociates into  $Na^+$  and  $NO_3^-$  ions, the positive sodium ions migrate into and through the electrically conductive glass of the lamp envelope 4 under the influence of the negative potential on the filament 6 due to source 20. Electrons emitted by the filament are attracted in the direction of the sodium supply by virtue of the positive potential of the source 20. At this stage in the process, the voltage of the source 20 becomes critical if the process of electrolysis is to continue with the neutralization of the sodium ions and the formation of a getter spot. Since the lamp is gas filled, an excessive number of the electrons from the filament can combine with gas ions if improper voltages are employed. As a result of this combination, positive sodium ions on the interior of the envelope are not neutralized and additional sodium ions will fail to enter the lamp by

virtue of the polarization effect at the inner wall thereof. The minimum value of the voltage of source 20 which overcomes polarization is 300 volts. Voltages below 300 are insufficient to avoid polarization by the migrated alkali ions. The variation of potential above the minimum voltage value is related to the type of lamp being gettered, the temperature of the filament, the pressure inside the lamp, the type of inert gas in the lamp and the distance between the filament and the lamp wall. As an example, using a cartridge lamp filled with argon to about 400 mm. Hg (at room temperature), a spacing of 4 mm. between the filament and lamp wall, a filament temperature of 2300° C., and a potential of 400 volts D.C. for source 20, there is a consistent neutralization of sodium to form the getter spot 24.

In FIG. 3 a cartridge lamp is shown with the greater spot 24 located on an inner portion of the envelope 4. The position of the spot 24 with regard to the remainder of the lamp envelope is precisely determined by the position of the probe 15 carrying the supply of the molten alkali compound. In addition, the area of the spot is directly related to the area of the supply of the molten compound carried by the probe 15 which is held in contact with the envelope during the process. The location and size of the spot is of particular importance in the gettering of a cartridge lamp where the getter spot must be small to permit full illumination from the lamp. The invention however is not limited to the gettering of cartridge type lamps.

I claim:

1. A method of providing a getter for a gas filled lamp, comprising the steps of:

- heating a portion of the selected glass envelope of a completed gas filled lamp to a temperature sufficient to cause the glass to become electrically conductive;
- placing the heated portion of the sealed lamp in contact with a supply of a molten alkali metal compound;
- initiating electron emission from the lamp filament into the envelope which is occupied by the inert gas;
- applying a potential across the lamp filament and the supply of molten alkali metal compound, said potential providing a sufficient voltage to bring about electrolytic conduction of the alkali metal through the heated portion of the glass envelope and to overcome polarization within the envelope; and
- discontinuing the application of said potential when a getter deposit of alkali metal is formed on a portion of the interior of the envelope adjacent the heated envelope surface which is in contact with the molten compound, said alkali metal being permanently retained within the glass envelope.

2. The method of providing a getter for a gas filled lamp according to claim 1 wherein the molten alkali metal compound is a eutectic mixture of sodium nitrate and sodium nitride and said getter deposit is sodium.

3. The method of providing a getter for a gas filled lamp according to claim 1 wherein said potential is at least 300 volts.

4. The method as in claim 1 wherein the lamp in which the getter deposit is formed is a cartridge type lamp.

#### References Cited

#### UNITED STATES PATENTS

|           |        |         |       |           |
|-----------|--------|---------|-------|-----------|
| 3,183,051 | 5/1965 | Schmidt | ----- | 316—3     |
| 3,189,395 | 6/1965 | Demas   | ----- | 313—222 X |

70 JAMES W. LAWRENCE, *Primary Examiner*.

DAVID O'REILLY, *Assistant Examiner*.

U.S. CL. X.R.

313—174, 179, 181

**U.S. DEPARTMENT OF COMMERCE**  
**PATENT OFFICE**  
**Washington, D.C. 20231**

**UNITED STATES PATENT OFFICE**  
**CERTIFICATE OF CORRECTION**

Patent No. 3,441,332

April 29, 1969

Nickolas P. Demas

It is certified that error appears in the above identified patent and that said Letters Patent are hereby corrected as shown below:

Column 4, line 32, "selected" should read -- sealed --.

Signed and sealed this 14th day of April 1970.

(SEAL)

Attest:

Edward M. Fletcher, Jr.

Attesting Officer

**WILLIAM E. SCHUYLER, JR.**

Commissioner of Patents